

## UNITED STATES PATENT OFFICE

2,668,113

## PHOTOGRAPHIC ANTIBRONZING AGENTS

Henry J. Schwalenstocker, Rochester, N. Y., assignor to E. I. du Pont de Nemours and Company, Wilmington, Del., a corporation of Delaware

No Drawing. Application January 26, 1951,  
Serial No. 208,058

9 Claims. (Cl. 95—7)

1

This invention pertains to photographic materials and more particularly to light-sensitive silver halide emulsions. Still more particularly it pertains to photographic silver halide emulsions which produce photographic silver images which do not degrade in color upon drying at elevated temperatures.

The practice of hot-drying or hot-ferotyping of photographic prints causes a degradation of the silver image characterized by an undesirable change in color. In the case of certain emulsions a loss in density also occurs. For instance, developed blue-black silver images usually degrade to a purplish or "plum" color and "warm-tone" images of basically brown color degrade to a green or black image upon hot-drying. Many compounds have been proposed for addition to photographic silver halide emulsions to prevent or reduce the color degradation described above. While some of the known materials reduce color degradation they have a strong desensitizing action which is disadvantageous. In addition, such compounds cause a degradation in the basic image color of "warm-tone" emulsions.

An object of the present invention is to provide photographic emulsions that yield developed silver images which do not undergo serious color degradation upon hot-drying. Another object is to provide such emulsions which are not desensitized by the adjuvants which prevent color degradation. A further object is to provide a simple and yet effective way of reducing color degradation by the addition of available chemical compounds. Still further objects will be apparent from the following description of the invention.

It has been found that the incorporation of salts of mercaptoazoles with N-hydrocarbon-substituted biguanides and especially N-aryl-substituted biguanides with photographic silver halide emulsions provide a high degree of color stabilization of the emulsions without any undesirable effect on the light-sensitive properties of the emulsions.

The salts referred to above may be represented by the general formula:



wherein R is hydrogen, or an alkyl or aryl group

2

and R' is an alkyl or aryl group Z constitutes the residue of a mercaptoazole. Thus, R and R' may be methyl, ethyl, propyl, isopropyl, isobutyl, phenyl, tolyl, naphthyl, etc., and HS—Z may be a mercaptoazole. Among the useful mercaptoazoles are 2-mercaptopbenzthiazole, 2-mercaptopbenzoxazole, and 5-mercaptotetrazole and their alkyl and aryl substituted derivatives, e. g., 1-phenyl-5-mercaptotetrazole, 1-a-naphthyl-5-mercaptotetrazole, 1-β-naphthyl-5-mercaptotetrazole, 1-p-diethylamino phenyl-5-mercaptotetrazole, 1-o-methoxy phenyl-5-mercaptotetrazole, 1-p-chlor phenyl-5-mercaptotetrazole, 2,5-dimercapto-1,3,4-thiadiazole, 1-benzyl-5-mercaptotetrazole, 1-cyclohexyl-5-mercaptotetrazole, 1-methyl-5-mercaptotetrazole and 1-ethyl-5-mercaptotetrazole.

The mercaptoazole salts of the N-hydrocarbon-substituted biguanides can be prepared by reacting the mercaptoazole and the N-aryl-biguanide in substantially equimolecular proportions in water or a methanol or ethanol solution and allowing the addition salts to crystallize.

Photographic silver images can be improved by the use of the novel salts described above by introducing them from an aqueous solution or an ethanol or methanol solution into the light-sensitive emulsion at some stage in its preparation prior to coating or into a subcoating or overcoating colloid composition, e. g., gelatin. Alternatively, the compounds may be incorporated in the photographic emulsion layer before or during development, e. g., by including them in the developing solution. They are preferably added to the photographic emulsion prior to coating.

In general, the salts are used in an amount of 0.1 to 1.0% by weight of the silver in the emulsion. When used in a gelatin overcoating or a developer solution or an ethanol or aqueous treating solution for the developed and fixed layer a similar or equivalent amount should be used.

The invention will be further illustrated but is not intended to be limited by the following examples.

## EXAMPLE I

One gram of phenylbiguanide mercaptobenzothiazole salt (A) was dissolved in 400 ml. of ethanol and this solution was added to a silver halide photographic emulsion composed of approximately 60% AgBr and 40% AgCl. The solution was added to the fluid emulsion immediately prior to coating in quantities varying between

80 and 400 ml. of solution per unit of emulsion where a unit is defined as that portion of emulsion containing 161.82 grams of silver. Control coatings were made from the same emulsion with no adjuvant and with 2-mercaptopbenzothiazole (B) added in the same quantities and according to the same procedure as described above.

An examination of photographic paper prints made from these coatings shows that while compound (A) causes an increase in warmth of basic image color, compound (B) causes a decrease in warmth of color. Comparison of coatings employing equal quantities of the two materials indicates that compound (A) is more effective than compound (B) in stabilizing image color on hot drying. The effect on sensitivity of the emulsion is noted in Table I.

Table I

| Adjuvant | Quantity Added <sup>1</sup> | Print Exposure Required <sup>2</sup> |
|----------|-----------------------------|--------------------------------------|
| A        | 80                          | 70                                   |
| A        | 200                         | 75                                   |
| A        | 400                         | 85                                   |
| B        | 80                          | 75                                   |
| B        | 200                         | 130                                  |
| B        | 400                         | 140                                  |
| None     |                             | 65                                   |

<sup>1</sup> Expressed in milliliters of solution per unit of emulsion.

<sup>2</sup> Expressed as relative time of exposure required to produce matched prints from a given negative. (Larger numbers indicate slower emulsion speed.)

## EXAMPLE II

A gelatin solution to be used as a protective coating which results in a final gelatin concentration of approximately 1% by weight was prepared in the usual manner. Quantities of phenylbiguanide 1-phenyl-5-mercaptopbenzothiazole salt (A) were added to the gelatin solution such that the final concentration of (A) in the gelatin solution ranged from 0.050 to 0.200 gram per liter. The resulting solutions were applied as a protective layer to a coating of photographic emulsion such as that described in Example I. Control coatings were made in which 1-phenyl-5-mercaptopbenzothiazole (B) was present in comparable quantities and in which no adjuvant was present.

Examination of normally- and hot-dried prints made from exposed photographic papers using these coatings in this case showed that compound B in all cases caused an undesirable loss in warmth of basic image color while compound A on the other hand increased warmth of basic image color. Further it was demonstrated that, while only 0.050 gram of compound A per liter of gelatin solution provided satisfactory color stability on hot drying, compound B did not provide this degree of stability when used in concentrations as high as 0.200 grams per liter of gelatin solution. The effect of these materials on emulsion sensitivity is noted in Table II.

Table II

| Adjuvant | Quantity Added <sup>1</sup> | Print Exposure Required <sup>2</sup> |
|----------|-----------------------------|--------------------------------------|
| A        | 0.05                        | 120                                  |
| A        | 0.10                        | 140                                  |
| A        | 0.20                        | 160                                  |
| B        | 0.05                        | 140                                  |
| B        | 0.10                        | 160                                  |
| B        | 0.20                        | 230                                  |
| None     |                             | 115                                  |

<sup>1</sup> Expressed in grams of material per liter of overcoating solution.

## EXAMPLE III

When photographic prints made from an exposed and developed printing paper made from an emulsion of the type described in Example I were immersed in a water solution of phenylbiguanide mercaptopbenzothiazole salt of 0.0005M concentration for one minute after normal processing it was found that color loss on hot drying was markedly decreased as compared to prints which did not receive such treatment.

## EXAMPLE IV

One gram of o-tolylbiguanide 1-phenyl-5-mercaptopbenzothiazole salt was dissolved in 400 ml. of ethanol and this solution was added to a silver halide photographic emulsion composed of approximately 60% AgBr and 40% AgCl. The solution was added to the emulsion immediately prior to coating in quantities varying between 200 and 800 ml. of solution per unit of emulsion.

Comparison of prints made from coatings of these emulsions with prints made on coatings of similar emulsion containing no adjuvant shows that this material provides a distinct improvement in image color of hot-dried prints.

## EXAMPLE V

Following the procedure of Example IV the following aryl biguanide salts were evaluated in the emulsion described in Example IV:

1. o-Tolylbiguanide mercaptopbenzothiazole salt.
2. o-Tolylbiguanide mercaptopbenzoxazole salt.
3. Phenylbiguanide 1-phenyl-5-mercaptopbenzothiazole salt.
4. Phenylbiguanide mercaptopbenzoxazole salt.

These compounds were all found to be effective in preventing loss of color on hot-drying of prints and gave results comparable with those described in Example IV with the o-tolylbiguanide 1-phenyl-5-mercaptopbenzothiazole salt.

## EXAMPLE VI

Photographic prints made on an emulsion of the type described in Example IV were immersed in a 0.0005M water solution of o-tolylbiguanide 1-phenyl-5-mercaptopbenzothiazole salt for one minute after normal processing. Other prints were treated in similar solutions of the compounds enumerated under Example V. Examination of the above prints after hot-drying as compared to untreated prints shows that color loss is reduced in each case where prints were treated in a solution of arylbiguanide salt.

## EXAMPLE VII

The following salts were prepared in ethanol such that the final concentration of solid salt in ethanol solution was of the order of 1 gram per 400 ml. of solution:

- (A) Phenyl biguanide - 2,5 - dimercapto - 1,3,4-thiadiazole
- (B) Biphenyl biguanide - 2,5 - dimercapto - 1,3,4-thiadiazole
- (C) Biphenyl biguanide-1-phenyl-5-mercaptopbenzothiazole.

The solutions were then added to respective emulsions of the kind described in Example I in quantities varying between 200 and 400 ml. of solution per unit of emulsion. These additions were made immediately prior to coating the light-sensitive emulsion onto a photographic paper support. In all cases the emulsions containing these salts were found to yield hot-dried prints

75

with image color superior to similar prints made from light-sensitive coatings made from similar emulsions free from such respective adjuvants.

In place of the specific hydrocarbon-substituted biguanide mercaptoazole salts described in the foregoing examples there may be substituted equivalent amounts of other such salts which fall within the scope of the above general formula. Among the additional salts which give similar results are: methyl, ethyl, phenyl and diphenyl biguanide 1-*a*-naphthyl-5-mercaptop-tetrazole or other substituted 5-mercaptop-tetrazole salts, 5-mercaptop 1,3,4-triazole salts, thio barbituric acid salts, salts of mercapto thiodiazoles and mercapto pyrimidines. Orthotolylbiguanide salts of the above mercapto compounds can also be used.

The compounds may be used in various types of emulsions which contain sensitizing dyes and other agents, e. g., anti-fogging agents, colloid-hardening agents, wetting and surface active agents, delusterants, etc. which modify the characteristics of an emulsion.

The invention is, of course, not limited to emulsions having gelatin as the water-permeable colloid for the silver halide binding agent or the overcoating or subcoating. Suitable additional colloids include agar-agar, polyglycuronic acids, zein, collodion, water-soluble cellulose derivatives, such as substantially hydrolyzed cellulose acetate, cellulose esters of hydroxy monocarboxylic acids, e. g., lactic or glycolic acids, alkali metal salts of cellulose esters of dicarboxylic acids, such as phthalic acid, polyvinyl alcohol, partially hydrolyzed polyvinyl acetate and interpolymers thereof with unsaturated materials, such as styrene, maleic acid, etc., water-soluble polyvinyl acetals and other hydrophilic synthetic or natural resins and polymeric compounds. Suitable hydrophilic colloids of the above types are described in United States Patents 2,110,491, 2,276,322, 2,276,323, 2,286,215 and 2,211,323.

An advantage of this invention is that it provides an effective way of reducing the color degradation of photographic images when subjected to hot-drying. Another advantage is that the adjuvants do not have any significant desensitizing effect on the light-sensitivity of the photographic emulsions. The use of phenylbiguanide 2-mercaptopbenzothiazole salt is especially advantageous in photographic warm-tone paper emulsions. A further advantage is that the salts have a high degree of solubility in methanol, ethanol and water which means that they can readily be associated with emulsions and photographic layers without the necessity of using expensive solvents and special procedures for their introduction into the photographic element. A still further advantage is that the adjuvants can be readily prepared from available chemicals.

As many widely different embodiments of this invention can be made without departing from the spirit and scope thereof, it is to be understood that the invention is not to be limited except as defined by the claims.

What is claimed is:

1. A photographic element comprising a support bearing a light-sensitive silver halide emul-

sion layer which contains a salt of a mercaptoazole with an N-hydrocarbon-substituted biguanide in an amount constituting 0.1% to 1.0% by weight of the silver in said emulsion.

5 2. A photographic element comprising a support bearing a light-sensitive silver halide emulsion layer which contains a salt of a mercaptoazole with an N-aryl-substituted biguanide in an amount constituting 0.1% to 1.0% by weight of the silver in said emulsion.

10 3. A photographic element comprising a paper base having a gelatino-silver-halide emulsion layer containing a salt of a mercaptoazole with an N-hydrocarbon-substituted biguanide in an amount constituting 0.1% to 1.0% by weight of the silver in said emulsion.

15 4. A photographic element comprising a paper base having a gelatino-silver-halide emulsion layer containing a salt of a mercaptoazole with an N-aryl-substituted biguanide in an amount constituting 0.1% to 1.0% by weight of the silver in said emulsion.

20 5. A photographic element comprising a paper base bearing a gelatino silver halide emulsion layer which contains a mercaptobenzothiazole salt of phenylbiguanide in an amount constituting 0.1% to 1.0% by weight of the silver in said emulsion.

25 6. The process of improving the color of a photographic silver image which comprises incorporating with the silver halide emulsion layer of a photographic paper prior to the completion of hot-drying a salt of a mercaptoazole with an N-hydrocarbon-substituted biguanide in an amount constituting 0.1% to 1.0% by weight of the silver in said emulsion.

30 7. The process of improving the color of a photographic silver image which comprises incorporating with the silver halide emulsion layer of a photographic paper prior to the completion of hot-drying a salt of a mercaptoazole with an N-aryl-substituted biguanide in an amount constituting 0.1% to 1.0% by weight of the silver in said emulsion.

35 8. A photographic silver halide emulsion containing a salt of a mercaptoazole with an N-hydrocarbon-substituted biguanide, in an amount constituting 0.1% to 1.0% by weight of the silver in said emulsion.

40 9. A photographic silver halide emulsion containing a salt of a mercaptoazole with an N-aryl-substituted biguanide, in an amount constituting 0.1% to 1.0% by weight of the silver in said emulsion.

45 50 55

HENRY J. SCHWALENSTOCKER.

References Cited in the file of this patent

UNITED STATES PATENTS

| Number    | Name            | Date          |
|-----------|-----------------|---------------|
| 1,725,934 | Reitstotter     | Aug. 27, 1929 |
| 1,763,989 | Sheppard et al. | June 17, 1930 |
| 2,317,184 | Dreyfuss        | Apr. 20, 1943 |
| 2,368,647 | Dreyfuss        | Feb. 6, 1945  |

FOREIGN PATENTS

| Number  | Country       | Date         |
|---------|---------------|--------------|
| 524,556 | Great Britain | Aug. 8, 1940 |
| 573,745 | Great Britain | Dec. 4, 1945 |